

## UNITED STATES PATENT OFFICE.

JOSEPH BENNETT, OF NORTH ADAMS, MASSACHUSETTS, ASSIGNEE TO CONSOLIDATED TEXTILE CORPORATION, OF NEW YORK, N. Y., A CORPORATION OF DELAWARE.

## FINISHED FABRIC AND PROCESS OF MAKING SAME.

No Drawing.

Application filed August 26, 1926. Serial No. 131,800.

This invention relates to artificial fibres and more particularly to the specialized treatment thereof for the purpose of improving the appearance.

5 It is well known that regenerated cellulose fibres, when they are made from xanthates or nitrates or from other intermediates, possess a fineness of fibre, a strength and softness which is highly desirable, but 10 they also possess a high lustre which for many purposes limits their application undesirably.

One of the objects of this invention is, therefore, to remove wholly or in part the 15 lustre from such fibres, while retaining their other desirable properties.

It has heretofore been customary, moreover, to manufacture fabrics from combinations of lustrous and lustreless fibres, in order to obtain desirable pattern effects. Such 20 manufacture, however, has required the use of a Jacquard loom, with all the consequent difficulties and expense.

It is a further object of this invention to 25 produce a process in accordance with which the lustre can be removed in localized areas from the finished fabric, whereby the pattern may be produced by printing rather than by weaving.

30 It is a further object to produce a process of the character described, which will be simple and efficient in operation and which will leave the fibres possessed of all their desirable properties and to produce a product which is highly ornamental and durable.

In accordance with this invention it has 35 been discovered that when the regenerated cellulose fibre is subjected to the action of a strong alkali, such for example as sodium hydrate, for a limited period, that the lustre is completely removed. This may in part be due to a hydration of the surface of individual fibres, or it may be a change in the physical condition of the surface thereof.

40 The process may be conducted generally for the purpose of producing a lustreless yarn or fabric, but it is particularly applicable to the forming of pattern effects, and for that reason I prefer to describe it more particularly as specifically so applied. When treating the fibre or the fabric as a whole, the fibre may be washed in a bath of sodium hydroxide for a limited time, depending upon the weight of the cloth, and thereafter submitted to such treatment as

will remove the remaining alkali by washing either with water or with a slightly acid bath.

When specifically applied to printing, the process is conducted as follows:—

The pattern is printed upon the fabric with a resist paste, as for example, a mixture of British gum and magnesium sulphate, it being understood, of course, that according to the general principles of resist printing, the pattern is in reverse, that is, the resist is placed upon those portions of the fabric which are to remain lustrous.

When the resist paste has become dried, the cloth is passed through a bath of sodium hydrate of a strength and temperature dependent upon the weight and thickness of the cloth and the effect desired. After which, the cloth is passed through a washing bath and preferably also a neutralizing bath such, for example, as a weak acid to eliminate the excess alkali.

As an alternative method, I may substitute for the resist paste a paste including a caustic soda mixed, for example, with gum tragacanth. This, when printed upon the fabric and allowed to remain during a light drying operation, is enough to remove the lustre from the fibre. The fabric is thereupon washed to remove the gum and neutralize the excess alkali. Either of the above processes will produce a pattern effect upon the cloth completely devoid of lustre at the spots acted upon by the reagents, but without affecting the lustre of the remaining portions of the goods.

Since certain changes may be made in carrying out the above process and in the product, and modifications effected in the apparatus for practicing the principle thereof, without departing from the scope of the invention, it is intended that all matter contained in the above description or shown in the accompanying drawing shall be interpreted as illustrative and not in a limiting sense.

It is also to be understood that the following claims are intended to cover all of the generic and specific features of the invention herein described, and all statements of the scope of the invention which, as a matter of language, might be said to fall therebetween.

I claim:

1. The process of ornamenting fabric of

60

65

70

75

80

85

90

95

100

105

110

2  
regenerated cellulose, which comprises subjecting the same to local treatment in pattern of caustic alkali of delustering strength.

5 2. The process of delusterizing the regenerated cellulose fibre, which comprises subjecting the same to the action of an alkali of delustering strength and subsequently neutralizing the remaining alkali.

10 3. The method of delusterizing regenerated cellulose fibre, which comprises washing the same in an alkaline bath of delustering strength, subsequently removing from the bath and neutralizing the excess alkali.

15 4. The process of ornamenting the regenerated cellulose, printing thereon with a paste in the desired pattern and subsequently subjecting said fabric to a bath, said paste or said bath including a caustic alkali.

20 5. The process of ornamenting a fabric of regenerated cellulose, which comprises printing thereon with a paste, including strong caustic, and thereafter removing said paste and neutralizing the remaining caustic.

25 6. The process of imposing a figure on cellulose fabrics which comprises forming a lustrous cellulose substitution product on localized areas.

7. The process of delustering regenerated cellulose fabrics, which comprises printing upon the fabric a substance capable of altering the surface of the fibres to remove gloss.

8. A fabric of regenerated cellulose fibre having localized area of lustreless surface.

9. A fabric of regenerated cellulose having localized lustreless areas formed by localized surface treatment of the fabric.

10. A fabric, individual fibres of which have an interior of reformed cellulose and a lustreless exterior of a cellulose substitution product.

11. The process of ornamenting a regenerated cellulose fabric, which comprises forming thereon a pattern of areas of glossed and unglossed fibres irrespective of the weave.

12. The process of ornamenting a regenerated cellulose fabric, which comprises forming thereon a pattern of unglossed cellulose substitution product irrespective of the weave.

In testimony whereof I affix my signature.

JOSEPH BENNETT.